

## UNITED STATES PATENT OFFICE

2,627,515

PRODUCTION OF ORGANIC ACID ESTERS  
OF CELLULOSE

Blanche B. White, Summit, and Peter Blackman, Westfield, N. J., assignors to Celanese Corporation of America, New York, N. Y., a corporation of Delaware

No Drawing. Application April 13, 1951,  
Serial No. 220,976

14 Claims. (Cl. 260—229)

1

This invention relates to the production of organic acid esters of cellulose and relates more particularly to an improved process for the production of organic acid esters of cellulose which may be carried out in a continuous manner.

In the production of organic acid esters of cellulose by the esterification of a cellulosic material, it is customary to pretreat the cellulosic material before esterification to increase its reactivity and thereby reduce the esterification time. To enable the production of the organic acid esters of cellulose to be carried out in a continuous manner, the pretreatment should require only a relatively short period of time. In addition, the pretreatment should increase the reactivity of the cellulosic material to a point where the esterification thereof will be completed rapidly.

It is an important object of this invention to provide a process for the production of organic acid esters of cellulose which will fulfill the foregoing requirements and which may be carried out in a continuous manner.

A further object of this invention is to provide a novel process for pretreating cellulosic material which may be carried out in a relatively short period of time and which will render said cellulosic material highly reactive.

Other objects of this invention will be apparent from the following detailed description and claims.

According to the present invention, a cellulosic material is pretreated with a mixture of a lower aliphatic acid and an acid cellulose esterification catalyst for the cellulosic material, said mixture containing from about 7.5 to 25 parts by weight of the acid cellulose esterification catalyst for each 100 parts by weight of the lower aliphatic acid, in the presence of from about 8 to 20 parts by weight of water for each 100 parts by weight of the lower aliphatic acid. The amount of water which must be present during the pretreatment may be in or may be added to the cellulosic material before the pretreatment begins, or it may be included in the pretreatment mixture, or a portion of the water may be in or may be added to the cellulosic material before the pretreatment begins and the remainder of the water may be included in the pretreatment mixture. It is preferred, however, to employ for the pretreatment

2 a cellulosic material containing at least about 4 parts by weight of water for each 100 parts by weight of the cellulosic material, since a cellulosic material containing a smaller quantity of water will not be rendered as reactive by the pretreatment as a cellulosic material containing at least this minimum quantity of water.

The best results and the most highly reactive cellulosic materials are obtained when the materials in the pretreatment mixture are employed in the ratio specified above and there is present during the pretreatment from about 4 to 7 parts by weight of water for each 100 parts by weight of the cellulosic material. In the case when this quantity of water, based on the cellulosic material, is present during the pretreatment, there should be employed from about 35 to 45 parts by weight of the lower aliphatic acid and from about 4 to 8 parts by weight of the acid cellulosic esterification catalyst for each 100 parts by weight of the cellulosic material to maintain the proper ratio of materials during the pretreatment.

The time required for the pretreatment of the cellulosic material under the conditions and with the materials specified is relatively short and the single stage of pretreatment yields a cellulosic material having an extremely high reactivity which may be esterified rapidly.

The process of the present invention may be applied to any suitable cellulosic material, such as cotton linters, or wood pulps or the like from which the lignin, pentosan, resins, and similar constituents have been removed, as for example, purified sulfite pulp, sulfate pulp or soda pulp. In addition, there may be employed cellulosic material derived from other sources such as bamboo, reeds, jute, esparto, straws such as linseed and hempseed straw, grasses, peanut hulls, bark, etc. The cellulosic material pretreated may be in the form of a mass of loose fibers, or in a form of a sheet, strip or board.

Any of the lower aliphatic acids including formic, acetic, propionic and butyric acids, as well as mixtures thereof, may be employed for the pretreatment of the cellulosic material. Similarly, any of the acid cellulose esterification catalysts may be employed with the lower aliphatic acid during the pretreatment, but it is preferred to employ sulfuric acid for this purpose since it is the cheapest and least hazardous cat-

alyst which produces a cellulosic material having a high reactivity in a short period of time.

The pretreatment mixture may be applied to the cellulosic material in any desired manner. For example, it may be sprayed or rolled onto the cellulosic material, or, when the cellulosic material is in the form of a sheet, strip or board, the pretreatment mixture may be applied thereto from a perforated or slotted conduit extending the full width of the sheet, strip or board. In 10 pretreating cellulosic material in the form of a mass of loose fibers, vigorous agitation should be provided during the application of the pretreatment mixture and during the first portion of the pretreatment period to insure a uniform distribution of the pretreatment mixture through the entire mass of material. Agitation of the cellulosic material should be continued during the entire pretreatment period, although less vigorous agitation may be employed during the latter stages thereof, it having been found that continuous agitation produces a more highly reactive cellulosic material as compared with a cellulosic material that is permitted to stand without agitation during a portion of the pretreatment period.

The temperature employed for the pretreatment is not critical and may range from about 20 to 50° C. A period of at least about 5 minutes or preferably between about 5 and 40 minutes should be allowed for the pretreatment to obtain a cellulosic material having the highest reactivity.

The pretreated cellulosic material is esterified with an organic acid anhydride, preferably employing an esterification mixture which contains additional quantities of lower aliphatic acid and which may also contain additional quantities of the esterification catalyst. The esterification mixture is advantageously cooled to freeze at least a portion of the lower aliphatic acid therein to prevent an excessive rise in temperature when the highly reactive cellulosic material is first contacted therewith. Esterification proceeds rapidly and is completed in about 15 to 30 minutes, or less. The lower aliphatic acid acts as a solvent for the organic acid ester of cellulose which is produced so that the product is obtained in the form of a clear dope. After the esterification is complete, a sufficient quantity of water may, as is well understood in the art, be added to the dope to convert any remaining organic acid anhydride to the corresponding acid, following which the organic acid ester of cellulose, preferably after the addition of a further quantity of water, may be permitted to hydrolyze or ripen to impart the desired solubility characteristics thereto. The organic acid ester of cellulose may then be precipitated from the dope, washed to free it from acids or other impurities, stabilized if necessary, washed again and finally dried. When organic acid esters of cellulose are prepared in accordance with the process of this invention, it is possible to carry out both the pretreatment and esterification on a continuous rather than on a batch basis, since the time required for both steps is sufficiently short to render a continuous process feasible.

Our invention will now be described specifically in connection with the production of cellulose acetate, which is commercially the most important organic acid ester of cellulose at the present time. It may, however, also be employed for the production of other organic acid esters of cellulose such as, for example, the lower aliphatic

acid esters of cellulose including cellulose propionate, cellulose butyrate, cellulose acetate propionate and cellulose acetate butyrate by substituting the corresponding organic acid anhydrides for the acetic anhydride employed in the production of cellulose acetate.

The following examples are given to illustrate this invention further.

#### Example I

Onto 100 parts by weight of cotton linters containing 6 parts by weight of water, there is sprayed a mixture containing 40 parts by weight of acetic acid and 6 parts by weight of sulfuric acid, and the cotton linters are stirred with rapid and efficient agitation for 15 minutes. The pretreated cotton linters are then esterified with an esterification mixture containing 250 parts by weight of acetic anhydride, 370 parts by weight of acetic acid and 7 parts by weight of sulfuric acid, which esterification mixture has been cooled to a temperature of 0° C. Esterification is complete in 16 minutes as evidenced by the clearing of the dope.

#### Example II

Onto 100 parts by weight of cotton linters containing 6 parts by weight of water, there is sprayed a mixture containing 35 parts by weight of acetic acid and 6 parts by weight of sulfuric acid, and the cotton linters are stirred with rapid and efficient agitation for 6 minutes. The pretreated cotton linters are then esterified with an esterification mixture containing 250 parts by weight of acetic anhydride, 330 parts by weight of acetic acid and 7 parts by weight of sulfuric acid, which esterification mixture has been cooled to 0° C. Esterification is complete in 16 minutes as evidenced by the clearing of the dope.

#### Example III

Onto 100 parts by weight of cotton linters containing 12 parts by weight of water, there is sprayed a mixture containing 80 parts by weight of acetic acid and 12 parts by weight of sulfuric acid, and the cotton linters are stirred with rapid and efficient agitation for 6 minutes. The pretreated cotton linters are then esterified with an esterification mixture containing 290 parts by weight of acetic anhydride and 240 parts by weight of acetic acid, which esterification mixture has been cooled to 0° C. Esterification is complete in 16 minutes as evidenced by the clearing of the dope.

#### Example IV

Onto 100 parts by weight of cotton linters containing 6 parts by weight of water, there is sprayed a mixture containing 40 parts by weight of acetic acid and 6 parts by weight of sulfuric acid, and the cotton linters are stirred slowly in a paddle mixer for 35 minutes. The pretreated cotton linters are then esterified with an esterification mixture containing 250 parts by weight of acetic anhydride, 330 parts by weight of acetic acid, and 7 parts by weight of sulfuric acid, which esterification mixture has been cooled to -6° C. Esterification is complete in 21 minutes as evidenced by the clearing of the dope.

It is to be understood that the foregoing detailed description is given merely by way of illustration and that many variations may be made therein without departing from the spirit of our invention.

Having described our invention, what we desire to secure by Letters Patent is:



parts by weight of acetic acid, in the presence of from about 8 to 20 parts by weight of water for each 100 parts by weight of the acetic acid, and esterifying the pretreated cellulosic material with acetic anhydride.

13. A process for the production of cellulose acetate from cellulosic material, which comprises pretreating a cellulosic material with a mixture of acetic acid and sulfuric acid, said mixture containing from about 4 to 8 parts by weight of sulfuric acid and from about 35 to 45 parts by weight of acetic acid for each 100 parts by weight of the cellulosic material in the presence of from about 4 to 7 parts by weight of water for each 100 parts by weight of the cellulosic material, and esterifying the pretreated cellulosic material.

14. A process for the production of cellulose acetate from cellulosic material, which comprises pretreating a cellulosic material containing at least about 4 parts by weight of water for each 100 parts by weight of the cellulosic material for a period of between about 5 and 40 minutes with

5 a mixture of acetic acid and sulfuric acid, said mixture containing from about 4 to 8 parts by weight of sulfuric acid and from about 35 to 45 parts by weight of acetic acid for each 100 parts by weight of the cellulosic material, in the presence of from about 4 to 7 parts by weight of water for each 100 parts by weight of the cellulosic material, and esterifying the pretreated cellulosic material.

10

15 BLANCHE B. WHITE.  
PETER BLACKMAN.

## REFERENCES CITED

The following references are of record in the file of this patent:

## UNITED STATES PATENTS

| Number    | Name             | Date          |
|-----------|------------------|---------------|
| 1,389,250 | Koetschet et al. | Aug. 30, 1921 |
| 1,425,581 | Esselen et al.   | Aug. 15, 1922 |
| 2,110,642 | Auden et al.     | Mar. 8, 1938  |
| 2,115,735 | Malm             | May 3, 1938   |
| 2,342,416 | Malm             | Feb. 22, 1944 |